

Aug. 12, 1941.

J. D. HANAWALT.

2,251,906

CONDENSATION OF MAGNESIUM VAPOR

Filed Jan. 29, 1940



Fig. 1



Fig. 2

INVENTOR

Joseph D. Hanawalt  
BY  
Griswold & Burdick  
ATTORNEYS

## UNITED STATES PATENT OFFICE

2,251,906

## CONDENSATION OF MAGNESIUM VAPOR

Joseph D. Hanawalt, Midland, Mich., assignor to  
The Dow Chemical Company, Midland, Mich.,  
a corporation of Michigan

Application January 29, 1940, Serial No. 316,199

5 Claims. (Cl. 75—67)

The invention relates to an improved method of condensing magnesium vapor.

The condensation of magnesium vapor to recover the metal substantially all in liquid form involves a number of serious practical difficulties, all resulting from the fact that liquid magnesium has a considerable vapor pressure. Thus, at ordinary condensation temperatures, particularly when operation is at considerably reduced pressure or in the presence of a large proportion of fixed gases, the vapor pressure of the condensed liquid magnesium, even at its solidification temperature, is an appreciable fraction of the partial pressure of the magnesium vapor to be condensed. Under these conditions the vapor can never be wholly liquefied in the condenser; some invariably escapes to cooler portions of the apparatus and collects as a fine powder, which is ordinarily not recovered. In addition, this dust, even if collected, cannot satisfactorily be melted down, but must be converted to massive magnesium by expensive methods.

An object of the present invention is to provide an improved method of condensing magnesium vapor. Another object is to provide a method in which the metal is substantially all converted into liquid form, even though the vapor is supplied under such conditions that the vapor pressure of the condensed liquid magnesium is an appreciable fraction of the partial pressure of the magnesium vapor.

According to the invention, magnesium vapor to be condensed is passed successively into two condensing zones, which are maintained at temperatures respectively above and below the melting point of magnesium. In the first zone most of the vapor is condensed to liquid magnesium, and in the second zone the remaining vapor is condensed to solid magnesium, usually in powder form. All the magnesium condensed is recoverable. If desired, condensate from the second zone may be returned into contact with the liquid condensate in the first zone where it melts and coalesces with the main body of condensed magnesium. In this way, substantially all the vapor condensed in both zones is finally obtained in the liquid state.

The invention may be explained in detail with reference to the accompanying drawing, in which:

Figure 1 is a vertical view, partly in section, of one form of apparatus adapted to carrying out the process of the invention; and

Figure 2 is a similar view of another form of apparatus.

The magnesium condenser shown in Figure 1 consists of a vertical elongated metal cylinder 11 provided with a vapor inlet 12 near its lower end and terminated at the bottom by a closed reservoir 13, which may be heated by an electric resistance element 14, and from which liquid metal can be withdrawn through double valves 15 and 16 with an intermediate receiver 17. The apparatus is closed at the top by a cover 18 provided with a gas outlet 19. The condenser 11 is divided into a lower zone A and an upper zone B which are cooled by radiation, and may be heated, if desired, by independent electric resistance windings 20 and 21. The vapor inlet 12, reservoir 13, and receiver 17 are covered with thermal insulation 22.

In operation, the reservoir 13 and the lower condensing zone A are raised to a temperature slightly above the melting point of magnesium by passing electric currents of suitable magnitude through their respective resistance windings 14 and 20. A stream of magnesium vapor is then introduced through the inlet 12. Most of the vapor is condensed in the lower zone A to a liquid metal, which flows down the walls of the condenser into the reservoir 13. The remaining vapor rises into the upper cooler condensing zone B where it deposits on the walls as a fine dust, some of which falls back into the pool of molten magnesium in the reservoir 13. Much of the magnesium dust being condensed clings to the wall of the condensing zone B, forming a deposit which increases in thickness and gradually lowers the rate of condensation in the zone. The deposit may be removed from time to time as necessary by passing electric current through the upper resistance winding 21, thus heating the walls of the zone B sufficiently to permit melting of the dust particles nearest the wall, causing the solid metal deposit to slide down the condenser into the reservoir 13. The dust, on reaching the reservoir fuses and coalesces satisfactorily with the main body of molten metal. Substantially all the magnesium vapor entering the condenser is recovered in liquid form, and may be tapped off as desired through the double valves 15 and 16. Any fixed gases present in the entering magnesium vapor escape through the upper outlet 19, to which suction may be applied if vacuum operation is desired.

In an alternative form of the apparatus shown in Figure 2, the magnesium dust depositing on the wall of the upper condensing zone B is continuously removed from the wall by means of a scraper 23 secured to a reciprocable shaft 24

mounted through the cover 18, and falls into the reservoir 13. In this case, an upper heating element adapted to dislodge the condensed powder is unnecessary.

The process of the invention may advantageously be applied to the condensation of magnesium vapor at any pressure, with or without the presence of accompanying gases such as hydrogen, helium, nitrogen, carbon monoxide, or hydrocarbon vapor. Such mixtures are formed in the production of magnesium by thermal reduction processes, and in the purification of magnesium metal by distillation. The new method is especially useful, however, when the magnesium vapor is supplied under such conditions of temperature, pressure, or dilution that the vapor pressure of the liquid magnesium in the condenser, even at its solidification temperature, is an appreciable fraction, say 3 per cent or more, of the pressure or partial pressure of magnesium in the vapor or vapor mixture to be condensed. It is under these conditions, especially when a vapor mixture is supplied at an absolute pressure below 100 mm. of mercury, that dust formation is most serious.

In practice the lower or liquid condensing zone A is maintained at any suitable condensing temperature above the melting point of magnesium (650° C.), usually in the range 660° C. to 750° C. The upper or solid condensing zone B is held preferably at a temperature sufficiently below the freezing point of magnesium that the vapor pressure of the solid condensed metal is negligible, temperatures of 50° C. to 500° C. being usual, and below 300° C. preferable.

It is not essential to the invention in the broadest form that the solid condensed magnesium dust be combined with the liquid condensate. Even when the two portions are separately withdrawn from the condenser, the recovery of magnesium is still higher than that attained in ordinary condensers. However, the return of the solid dust to the liquid condensate is a very great advantage, since it permits recovery of substantially all of the condensate in the liquid state.

It is to be understood that the foregoing description is illustrative rather than strictly limitative, and that the invention is co-extensive in scope with the following claims.

I claim as my invention:

1. A method of condensing magnesium vapor which comprises passing the vapor successively into two condensation zones maintained at condensation temperatures respectively above and below the melting temperature of magnesium, whereby the major portion of the vapor is condensed in the first zone directly to a liquid and the remaining vapor is condensed in the second zone as a solid, and combining the condensate from the second zone with that formed in the first zone, whereby substantially all the magnesium condensed is recovered in the liquid state.

2. In a method of condensing magnesium vapor wherein the vapor is supplied under such conditions of temperature and pressure that the vapor pressure of the condensed liquid magnesium formed in the process is an appreciable fraction of the partial pressure of the magnesium vapor to be condensed, the steps which comprise passing the vapor successively into two condensation zones, the first being maintained at a condensing temperature above the melting temperature of magnesium and the second maintained at a temperature such that the vapor pressure of magnesium at that temperature is negligible, and combining the condensate from the second zone with that formed in the first zone, whereby substantially all the magnesium condensed is recovered in the liquid state.

3. In a method of condensing magnesium vapor from admixture with fixed gases, the mixture being supplied under such conditions of temperature and pressure that the vapor pressure of the condensed liquid magnesium formed in the process is an appreciable fraction of the partial pressure of the magnesium vapor to be condensed, the steps which comprise passing the vapor successively into two condensation zones, the first being maintained at a condensing temperature above the melting temperature of magnesium, and the second maintained at a temperature such that the vapor pressure of magnesium at that temperature is negligible, and combining the condensate from the second zone with that formed in the first zone, whereby substantially all the magnesium condensed is recovered in the liquid state.

4. A method of condensing magnesium vapor from admixture with fixed gases, the mixture being supplied at an absolute pressure below 100 mm. of mercury, which comprises passing the mixture successively into two condensation zones, the first being maintained at a temperature between about 660° C. and about 750° C., and the second at a temperature between about 50° C. and about 500° C., and combining the condensate from the second zone with that formed in the first zone, whereby substantially all the magnesium condensed is recovered in the liquid state.

5. In a method of condensing magnesium vapor, the steps which comprise passing the vapor successively into two condensation zones, the first being maintained at a temperature between about 660° and about 750° C. and the second at a temperature between about 50° and about 500° C., whereby the major portion of the vapor is condensed in the first zone directly to a liquid and the remaining vapor is condensed in the second zone as a solid, and combining the condensate from the second zone with that from the first zone, whereby substantially all of the magnesium condensed is recovered in the liquid state.

JOSEPH D. HANAWALT.